

# UNITED STATES PATENT OFFICE.

MORDUCH L. KAPLAN, OF BROOKLYN, NEW YORK. \*

## GALVANIC CELL.

1,109,129.

Specification of Letters Patent. Patented Sept. 1, 1914.

No Drawing.

Application filed June 1, 1914. Serial No. 842,021.

To all whom it may concern:

Be it known that I, MORDUCH L. KAPLAN, a citizen of the United States, and a resident of Brooklyn, in the county of Kings and State of New York, have invented certain new and useful Improvements in Galvanic Cells, of which the following is a specification.

The object of the present invention is to provide a good depolarizer for the galvanic cell of the Leclanché type.

I have discovered that blue hydrated potassium manganite when treated with a dilute solution of a manganous salt, is changed into a dark colored manganous polymanganite according to the following equation:



I have further discovered that this hy-

drated manganous polymanganite when heated in the air, can be made to lose nearly all its water without any appreciable loss of oxygen. Both products, the hydrated as 25 well as the dehydrated, are deep, bluish-dark colored, fine dense powders, excellent depolarizers, and give good results when used in the Leclanché cell, in relation to yield and steadiness of current. 30

What I claim as my invention and desire to secure by Letters Patent, is:

A galvanic cell containing manganous polymanganite as a depolarizing agent.

Signed at New York city, in the county of 35 New York and State of New York, this 29th day of May A. D. 1914.

MORDUCH L. KAPLAN.

Witnesses:

ARTHUR MARION,  
CHAS. C. GILL.